

# United States Patent Office

2,848,393

Patented Aug. 19, 1958

1

2,848,393

## BRIGHT CADMIUM PLATING

Donald Gardner Foulke, Watchung, and Otto Kardos, Red Bank, N. J., assignors to Hanson-Van Winkle-Munning Company, a corporation of New Jersey

No Drawing. Application November 8, 1955  
Serial No. 545,778

10 10 Claims. (Cl. 204—50)

This invention relates to bright cadmium plating, and provides an improved process and improved cadmium plating bath for producing bright or brilliant cadmium electrodeposits over a wide current density range.

We have found that bright and even brilliant electrodeposits of cadmium may be formed from a conventional alkali cyanide cadmium plating bath by incorporating in such bath a fraction of a gram per liter of a water-dispersible cellulose derivative together with a small amount of an alkylene or polyalkylene glycol or an alkyl ether derivative of such glycol. Accordingly, the process of this invention for producing bright cadmium deposits comprises electrodepositing cadmium from an aqueous alkaline solution containing from 50 to 150 grams per liter of an alkali metal cyanide, from 10 to 50 grams per liter of cadmium, from  $\frac{1}{100}$  to  $\frac{3}{4}$  gram per liter of a water-dispersible cellulose derivative, and from  $\frac{1}{4}$  to 30 grams per liter of a glycolic compound having the formula



in which R is a substituent selected from the group consisting of hydrogen and alkyl radicals containing from 1 to 6 carbon atoms, X is a substituent selected from the group consisting of hydrogen, methyl and ethyl, and n is a number from 0 to 500. Advantageously the process of our invention is carried out using an alkali cyanide cadmium plating bath in which the concentration of cyanide and of cadmium, and the ratio of cyanide concentration to cadmium concentration, are within the ranges generally considered optimum in ordinary cadmium electroplating operations. Thus, the plating bath advantageously contains from 65 to 130 grams per liter of an alkali metal cyanide and from 15 to 35 grams per liter of cadmium; and generally we prefer to employ from  $\frac{1}{100}$  to  $\frac{1}{2}$  gram per liter of the water-dispersible cellulose derivative, together with from 1 to 4 grams per liter of the glycolic compound.

Any cellulose derivative which can be dispersed in the plating bath, i. e. any water-dispersible cellulose derivative, may be employed in carrying out the method of this invention. We have obtained particularly satisfactory results, however, using as the cellulose derivative one selected from the group consisting of hydroxyethyl cellulose, carboxymethyl cellulose, and hydroxyethyl carboxymethyl cellulose.

The glycolic compound used in carrying out the method of the invention is of course a compound of the group consisting of alkylene glycols, polyalkylene glycols, and

5

10

20

25

30

35

40

45

50

55

60

2

alkyl ether derivatives of such glycols. The alkylene and polyalkylene glycols used are preferably those in which the alkyl unit (i. e. CH<sub>2</sub> in the general formula given above) contains from 1 to 3 carbon atoms. The polyalkylene glycols differ from the alkylene glycols in that the former contain a plurality, up to about 500, alkyl units, whereas the latter contain only one, i. e. n equals zero in the general formula given above. The alkyl ether derivatives of said glycols preferably are compounds in which the terminal alkyl substituents, i. e. R in the general formula given above, contain 1 to 6 carbon atoms.

Although excellent bright cadmium electroplates may be deposited from a bath containing only the cellulose derivative and the glycolic compound as addition agents, we have found that it is generally possible to improve the brilliance of the electroplate, and particularly to broaden the current density range over which bright deposits are formed, by incorporating a fraction of a gram per liter of dissolved nickel in the plating bath. In general, from  $\frac{1}{1000}$  to  $\frac{3}{4}$  gram per liter of nickel may be employed effectively, but ordinarily we prefer that the amount of nickel incorporated in the bath be in the narrower range from  $\frac{1}{100}$  to  $\frac{1}{2}$  gram per liter. The nickel may be introduced into the bath by dissolving therein any nickel salt which is soluble in the bath and which does not incorporate an anion having an adverse effect on the operation of the bath.

A conventional alkali cyanide plating bath, to which the above-identified addition agents may be added for making up a plating bath in accordance with this invention customarily is of the following composition:

|                             | Ounces per Gallon | Grams per Liter |
|-----------------------------|-------------------|-----------------|
| Cadmium (as metal).....     | 2.0 to 4.5        | 15 to 35        |
| Sodium Cyanide (total)..... | 8.5 to 17.5       | 65 to 130       |
| Sodium Hydroxide.....       | 1.0 to 3.2        | 7.5 to 25       |
| Sodium Carbonate.....       | 0 to 15           | 0 to 110        |

A typical alkali cyanide cadmium plating solution is made by dissolving 3.5 ounces per gallon of cadmium oxide and 15.0 ounces per gallon of sodium cyanide in water. The solution thus formed is rendered alkaline by the caustic soda formed by reaction of cadmium oxide and sodium cyanide in the aqueous solution. A bath of this basic composition was employed in carrying out the examples of the invention that are summarized in Tables I to IV below.

Table I below sets forth a considerable number of glycolic addition agents which have been used successfully in the process of this invention. Table I further summarizes the results obtained when an electrodeposit was formed from a solution having the above specified basic composition and containing 0.08 gram per liter of hydroxyethyl cellulose. The electrodeposit was formed in a Hull test cell on sheet steel cathodes, at room temperature and at a total current of 1 ampere, and with a plating time of ten minutes. Each glycolic compound was used in a plating solution containing no nickel, and again in a solution containing 0.02 gram per liter of nickel added in the form of nickel sulfate to the plating bath.

Table I

|     | Glycolic Compound                        |              | Nickel Conc., g./l. | Results                       |                             |
|-----|------------------------------------------|--------------|---------------------|-------------------------------|-----------------------------|
|     | Name                                     | Conc., g./l. |                     | Brightness                    | Bright Current Density Area |
| 1.  | Diethylene glycol monoethyl ether        | 6            | Bright              | low and middle.               |                             |
| 2.  |                                          | 10           | do                  | middle and high.              |                             |
| 3.  |                                          | 2            | do                  | all but lower $\frac{1}{4}$ . |                             |
| 4.  | Diethylene glycol monobutyl ether        | 2            | Very Bright         | overall.                      |                             |
| 5.  |                                          | 1            | Bright              | Do.                           |                             |
| 6.  | Diethylene glycol dibutyl ether          | 1            | do                  | Do.                           |                             |
| 7.  |                                          | 1            | do                  | low and middle.               |                             |
| 8.  | Diethylene glycol hexylether             | 1            | do                  | Do.                           |                             |
| 9.  | Ethylene glycol                          | 1            | do                  | middle $\frac{1}{4}$ .        |                             |
| 10. |                                          | 4            | do                  | middle 60%.                   |                             |
| 11. | Diethylene glycol                        | 1            | do                  | middle $\frac{1}{4}$ .        |                             |
| 12. |                                          | 48           | do                  | overall, some smut.           |                             |
| 13. | Triethylene glycol                       | 1            | do                  | middle $\frac{1}{4}$ .        |                             |
| 14. |                                          | 6            | do                  | all except low 10%.           |                             |
| 15. | Propylene glycol                         | 1            | do                  | middle $\frac{1}{4}$ .        |                             |
| 16. |                                          | 8            | do                  | middle 60%.                   |                             |
| 17. | Dipropylene glycol                       | 1            | do                  | middle 40%.                   |                             |
| 18. |                                          | 8            | do                  | overall.                      |                             |
| 19. | Methoxy propylene glycol                 | 0.1          | do                  | overall, some haze.           |                             |
| 20. |                                          | 0.1          | Brilliant           | Do.                           |                             |
| 21. | Ethoxy triethylene glycol                | 1            | Bright              | middle $\frac{1}{2}$ .        |                             |
| 22. |                                          | 2            | do                  | overall, some haze.           |                             |
| 23. | Ethylene glycol ethyl ether              | 16           | do                  | upper $\frac{1}{4}$ .         |                             |
| 24. |                                          | 16           | do                  | Do.                           |                             |
| 25. | Ethylene glycol diethyl ether            | 12           | do                  | middle $\frac{1}{4}$ .        |                             |
| 26. |                                          | 12           | Fairly Bright       | overall                       |                             |
| 27. | Ethylene glycol 2-ethyl butyl ether      | 1            | Bright              | middle $\frac{1}{2}$ .        |                             |
| 28. |                                          | 3            | Brilliant           | Do.                           |                             |
| 29. | Ethylene glycol hexyl ether              | 0.1          | Bright              | low 40%.                      |                             |
| 30. |                                          | 0.24         | do                  | all except very low.          |                             |
| 31. | Ethylene glycol butyl ether              | 4            | do                  | middle $\frac{1}{2}$ .        |                             |
| 32. |                                          | 4            | do                  | low and middle.               |                             |
| 33. | Ethylene glycol methyl ether             | 1            | do                  | middle $\frac{1}{4}$ .        |                             |
| 34. |                                          | 40           | Hazy Bright         | high $\frac{1}{4}$ .          |                             |
| 35. | Diethylene glycol monovinyl ether        | 0.1          | Bright              | middle $\frac{1}{4}$ .        |                             |
| 36. |                                          | 12           | do                  | middle $\frac{1}{4}$ .        |                             |
| 37. | Dibutoxy Tetra glycol                    | 0.01         | do                  | low 40%.                      |                             |
| 38. |                                          | 0.04         | do                  | overall, some haze.           |                             |
| 39. | Polyethylene glycol, av. mol. wt. 300    | 1.0          | do                  | overall.                      |                             |
| 40. |                                          | 1.0          | do                  | Do.                           |                             |
| 41. | Polyethylene glycol, av. mol. wt. 400    | 0.1          | do                  | overall, some haze.           |                             |
| 42. |                                          | 0.1          | do                  | overall, slight haze.         |                             |
| 43. | Polyethylene glycol, av. mol. wt. 600    | 0.1          | do                  | Do.                           |                             |
| 44. |                                          | 0.1          | do                  | Do.                           |                             |
| 45. | Polyethylene glycol, av. mol. wt. 1,000  | 0.1          | Brilliant           | upper $\frac{1}{2}$ .         |                             |
| 46. |                                          | 0.1          | Bright              | upper $\frac{1}{4}$ .         |                             |
| 47. | Polyethylene glycol, av. mol. wt. 3,400  | 0.01         | do                  | lower $\frac{1}{4}$ .         |                             |
| 48. |                                          | 0.01         | do                  | middle $\frac{1}{2}$ .        |                             |
| 49. | Polyethylene glycol, av. mol. wt. 6,800  | 0.01         | do                  | low and high.                 |                             |
| 50. |                                          | 0.01         | do                  | upper $\frac{1}{2}$ .         |                             |
| 51. | Polyethylene glycol, av. mol. wt. 20,000 | 0.01         | do                  | upper $\frac{1}{4}$ .         |                             |
| 52. |                                          | 0.01         | do                  | upper $\frac{1}{2}$ .         |                             |
| 53. | Polypropylene glycol, av. mol. wt. 400   | 0.1          | Brilliant           | upper 60%.                    |                             |
| 54. |                                          | 0.1          | Bright              | overall, some streaks.        |                             |
| 55. | Tetraethylene glycol dimethyl ether      | 2            | do                  | middle $\frac{1}{2}$ .        |                             |
| 56. |                                          | 4            | do                  | middle and upper.             |                             |

Of the various glycolic compounds which may be used in accordance with the method of this invention, we have obtained particularly satisfactory results using butyl ether derivatives of ethylene glycol. Diethylene glycol monobutyl ether, for example, has been found to be a particularly effective brightener over a very wide current density range, and we therefore consider this compound to be especially suitable for commercial use in bright cadmium plating according to this invention. Excellent results also are obtained, as indicated in Table I, when using diethylene glycol dibutyl ether, and when using ethylene glycol 2-ethyl butyl ether.

Our experience has indicated that any water-dispersible cellulose derivative may be used effectively in bright cadmium plating baths prepared according to our invention.

Table II below summarizes a number of examples of the method of this invention in which different cellulose derivatives were used. The results of Table II were obtained by electroplating cadmium from a solution having the basic composition given above and to which 2 grams per liter of diethylene glycol monobutyl ether had been added. The cadmium was electroplated from the solution in a Hull test cell at a total current of 1 ampere and at room temperature. The various cellulose derivatives set forth in Table II were dispersed in the solution in the concentrations indicated. Each cellulose compound was tested in a solution free from nickel, and again in a solution to which 0.02 gram per liter of nickel, added as nickel sulfate, had been dissolved.

Table II

| Cellulose Derivative                 | Name | Nickel Conc., g./l. | Results        |                             |
|--------------------------------------|------|---------------------|----------------|-----------------------------|
|                                      |      |                     | Brightness     | Bright Current Density Area |
| Hydroxyethyl cellulose               |      | 0.1                 | Bright         | overall, except lower 15%.  |
|                                      |      | 0.1                 | Very Bright    | overall.                    |
| Carboxymethyl cellulose              |      | 0.12                | Bright         | low and high.               |
|                                      |      | 0.12                | do             | overall, except very low.   |
| Carboxymethyl-hydroxyethyl cellulose |      | 0.1                 | Bright         | Do.                         |
|                                      |      | 0.1                 | Very Bright    | Do.                         |
| Oxidized cellulose                   |      | 0.01                | Dullish Bright | overall.                    |
|                                      |      | 0.12                | Brilliant      | upper $\frac{1}{4}$ .       |

It will be noted from the foregoing table that oxidized cellulose, when used in the solution containing no nickel and at the minimum preferred concentration, resulted in the electrodeposit being less bright than was the case in the other tests. However, when the concentration of the oxidized cellulose was increased to a value well within the preferred range, and when it was used in the presence of dissolved nickel, it resulted in an exceptionally bright deposit in the higher current density range. Since performance of this material seems to be more dependent on concentration and on other factors than the first three compounds listed in Table II, it is relatively less satisfactory than the latter for commercial use.

The wide concentration range of the glycolic compound and the wide current density range over which bright deposits can be obtained by the method of this invention is illustrated in Table III below. In carrying out the examples summarized in Table III, 0.1 gram per liter of hydroxyethyl cellulose and 0.02 gram per liter of nickel (added as nickel sulfate) were incorporated in an alkali cyanide cadmium solution of the basic composition stated above. Diethylene glycol monobutyl ether was added to the solution in the amounts indicated in the table, and cadmium was plated from the solution at room temperature, without agitation, on steel cathodes immersed in the bath.

Table III

| Diethylene Glycol Monobutyl Ether Conc., g./l. | Brightness of Cathode Deposit at Current Density of |                              |                      |
|------------------------------------------------|-----------------------------------------------------|------------------------------|----------------------|
|                                                | 10 Amps. per sq. ft.                                | 25 Amps. per sq. ft.         | 40 Amps. per sq. ft. |
| 1/2                                            | Bright with smut                                    | Bright                       | Bright               |
| 1                                              | Bright, some smut                                   | do                           | Do.                  |
| 2                                              | Dullish bright                                      | Very Bright                  | Very Bright.         |
| 4                                              | do                                                  | do                           | Bright.              |
| 12                                             | do                                                  | Bright, Lacking Full Luster. | Dullish Bright.      |

Table III indicates that for optimum results the current density from 20 to 40 amperes per square foot should be used. In particular, low current densities of about 10 amperes per square foot or less give less satisfactory bright deposits than are obtained at the higher current densities. However, even at low current densities, a degree of brightening which is useful for many purposes can be obtained.

As shown in Table IV below, the concentration of the cellulose derivative, within the preferred range contemplated by the invention, and particularly in the presence of dissolved nickel, is not critical. In carrying out the examples summarized in Table IV, 2 grams per liter of diethylene glycol monobutyl ether were dissolved in an alkali cadmium cyanide solution having the basic composition stated above. Hydroxyethyl cellulose was dissolved in the resulting solution at concentrations indicated in Table IV, and nickel sulfate was also dissolved therein to yield the nickel concentrations indicated. Cadmium was electrodeposited from the resulting solution at room temperature, without agitation, on steel cathodes, and the character of the electrodeposit formed at various current densities was noted.

Table IV

| Hydroxyethyl Cellulose Conc., g./l. | Nickel Conc., g./l. | Current Density, Amps. per sq. ft. | Character of Deposit                                    |
|-------------------------------------|---------------------|------------------------------------|---------------------------------------------------------|
| 0.01                                | 0.02                | 25 to 40                           | Very Bright.                                            |
| 0.1                                 | 0.02                | 15 to 50                           | Brilliant.                                              |
| 0.4                                 | 0.02                | 25 and 40                          | Bright.                                                 |
| 0.8                                 | 0.02                | 10 to 40                           | Dullish Bright, some smut.                              |
| 0.1                                 | 0.01                | 25 to 40                           | Bright.                                                 |
| 0.1                                 | 0.40                | 25 and 40                          | Bright. Bright at 25 a. s. f., some haze at 40 a. s. f. |

We claim:

1. A process for producing bright cadmium deposits which comprises electrodepositing cadmium from an aqueous alkaline solution containing from 50 to 150 grams per liter of an alkali metal cyanide, from 10 to 50 grams per liter of cadmium, from  $\frac{1}{1000}$  to  $\frac{1}{4}$  gram per liter of a water-dispersible cellulose derivative, and from  $\frac{1}{4}$  to 30 grams per liter of a glycolic compound having the formula



in which R is a substituent selected from the group consisting of hydrogen and alkyl radicals containing from 1 to 6 carbon atoms, X is a substituent selected from the group consisting of hydrogen, methyl, and ethyl, and n is a number from 0 to 500.

2. A process for producing bright cadmium deposits which comprises electrodepositing cadmium from an aqueous alkaline solution containing from 65 to 130 grams per liter of an alkali metal cyanide, from 15 to 35 grams per liter of cadmium, from  $\frac{1}{100}$  to  $\frac{1}{2}$  gram per liter of a water-dispersible cellulose derivative, and from 1 to 4 grams per liter of a glycolic compound having the formula



in which R is a substituent selected from the group consisting of hydrogen and alkyl radicals containing from 1 to 6 carbon atoms, X is a substituent selected from the group consisting of hydrogen, methyl, and ethyl, and n is a number from 0 to 500.

3. A process for producing bright cadmium deposits which comprises electrodepositing cadmium from an aqueous alkaline solution containing from 50 to 150 grams per liter of an alkali metal cyanide, from 10 to 50 grams per liter of cadmium, from  $\frac{1}{1000}$  to  $\frac{1}{4}$  gram per liter of nickel, from  $\frac{1}{1000}$  to  $\frac{1}{4}$  gram per liter of a water-dispersible cellulose derivative, and from  $\frac{1}{4}$  to 30 grams per liter of a glycolic compound having the formula



in which R is a substituent selected from the group consisting of hydrogen and alkyl radicals containing from 1 to 6 carbon atoms, X is a substituent selected from the group consisting of hydrogen, methyl, and ethyl, and n is a number from 0 to 500.

4. A process for producing bright cadmium deposits which comprises electrodepositing cadmium from an aqueous alkaline solution containing from 65 to 130 grams per liter of an alkali metal cyanide, from 15 to 35 grams per liter of cadmium, from  $\frac{1}{100}$  to  $\frac{1}{2}$  gram per liter of nickel, from  $\frac{1}{100}$  to  $\frac{1}{2}$  gram per liter of a water-dispersible cellulose derivative, and from 1 to 4 grams per liter of a glycolic compound having the formula



in which R is a substituent selected from the group consisting of hydrogen and alkyl radicals containing from 1 to 6 carbon atoms, X is a substituent selected from the group consisting of hydrogen, methyl, and ethyl, and n is a number from 0 to 500.

5. A process for producing bright cadmium deposits which comprises electrodepositing cadmium from an aqueous alkaline solution containing from 65 to 130 grams per liter of an alkali metal cyanide, from 15 to 35 grams per liter of cadmium, from  $\frac{1}{100}$  to  $\frac{1}{2}$  gram per liter of a cellulose derivative selected from the group consisting of hydroxyethyl cellulose, carboxymethyl cellulose, and hydroxyethyl carboxymethyl cellulose, and from 1 to 4 grams per liter of an ether derivative of a compound selected from the group consisting of alkylene glycols and polyalkylene glycols.

6. A process for producing bright cadmium deposits which comprises electrodepositing cadmium from an aqueous alkaline solution containing from 65 to 130 grams per liter of an alkali metal cyanide, from 15 to 35 grams per liter of cadmium, from  $\frac{1}{100}$  to  $\frac{1}{2}$  gram per liter of a cellulose derivative selected from the group consisting of hydroxyethyl cellulose, carboxymethyl cellulose, and hydroxyethyl carboxymethyl cellulose, and from 1 to 4 grams per liter of a compound selected from the group consisting of alkylene glycols and polyalkylene glycols.

7. A process for producing bright cadmium deposits which comprises electrodepositing cadmium from an aqueous alkaline solution containing from 65 to 130 grams per liter of an alkali metal cyanide, from 15 to 35 grams per liter of cadmium, from  $\frac{1}{100}$  to  $\frac{1}{2}$  gram per liter of nickel, from  $\frac{1}{100}$  to  $\frac{1}{2}$  gram per liter of hydroxyethyl cellulose, and from 1 to 4 grams per liter of diethylene glycol butyl ether.

8. An aqueous alkali-cyanide cadmium plating bath containing from 50 to 150 grams per liter of an alkali metal cyanide, from 10 to 50 grams per liter of cadmium, from  $\frac{1}{1000}$  to  $\frac{3}{4}$  gram per liter of a water-dispersible cellulose derivative, and from  $\frac{1}{4}$  to 30 grams per liter of a glycolic compound having the formula



in which R is a substituent selected from the group consisting of hydrogen and alkyl radicals containing from 1 to 6 carbon atoms, X is a substituent selected from the

10

15

20

25

30

group consisting of hydrogen, methyl, and ethyl, and n is a number from 0 to 500.

9. An aqueous alkali-cyanide cadmium plating bath containing from 65 to 130 grams per liter of an alkali metal cyanide, from 15 to 35 grams per liter of cadmium, from  $\frac{1}{100}$  to  $\frac{1}{2}$  gram per liter of nickel, from  $\frac{1}{100}$  to  $\frac{1}{2}$  gram per liter of a water-dispersible cellulose derivative, and from 1 to 4 grams per liter of a glycolic compound having the formula



in which R is a substituent selected from the group consisting of hydrogen and alkyl radicals containing from 1 to 6 carbon atoms, X is a substituent selected from the group consisting of hydrogen, methyl, and ethyl, and n is a number from 0 to 500.

10. An aqueous alkali cyanide plating bath containing from 65 to 130 grams per liter of an alkali metal cyanide, from 15 to 35 grams per liter of cadmium, from  $\frac{1}{100}$  to  $\frac{1}{2}$  gram per liter of nickel, from  $\frac{1}{100}$  to  $\frac{1}{2}$  gram per liter of hydroxyethyl cellulose, and from 1 to 4 grams per liter of diethylene glycol butyl ether.

#### References Cited in the file of this patent

#### UNITED STATES PATENTS

|           |                         |               |
|-----------|-------------------------|---------------|
| 2,107,806 | Solderberg et al. ----- | Feb. 8, 1938  |
| 2,526,999 | Diggin et al. -----     | Oct. 24, 1950 |
| 2,615,837 | Liger -----             | Oct. 28, 1952 |